

## UNITED STATES PATENT OFFICE

EARL P. STEVENSON, OF NEWTON, MASSACHUSETTS, ASSIGNOR TO THE RICHARDSON COMPANY, OF LOCKLAND, OHIO, A CORPORATION OF OHIO

FIBROUS COMPOSITION CONTAINING FILLER AND BINDER SUBSTANCES AND PROCESS OF MAKING THEM

No Drawing.

Application filed April 6, 1931. Serial No. 528,248.

My present invention is concerned with the manufacture of fibrous compositions and articles containing organic binders and mineral or other fillers, wherein the fiber distribution and construction is characteristic of a paper mill product, and is more particularly related to the preparation of a watery pulp in which fiber, binder and filler are intimately associated. Broadly, in 10 the practice of my invention I employ a basic principle which was set forth in United States Patent No. 1,771,150, of July 22, 1930. This principle applies to the manufacture of pulps suitable for formation on a screen by 15 a method which comprises first pre-associating a binder substance and a fibrous material while the fibers are not in water suspension in the sense of constituting a pulp, and after such pre-association has been produced, 20 then suspending the fibrous material and the associated binder substance in water sufficient to act as a circulating medium, and refining the stock for felting.

It has been found possible to produce a 25 relationship or pre-association between fibers and a binder substance even in large amounts of the latter, which pre-association is not wholly destroyed in any subsequent treatments which the fibrous material receives, such as in beating or Jordaning, to 30 prepare them for felting upon a screen. The stability of the association is apparently a residual function of the pre-association of the fibers and the binder substance.

In a co-pending application, Serial No. 35 468,454, filed July 16, 1930, in the names of Stevenson and Buron, there has been described and claimed a procedure employing the same general principle, but directed to 40 the production of articles in which a synthetic resinous material is associated with the fibers. My present invention is distinguished in point of novelty from the patent and application hereinabove mentioned, by 45 the manner in which the filler is incorporated, and by the adhesive relationship here obtained between an organic binder and a mineral filler, whereby new and useful results are produced.

50 My present process permits of the use of

various kinds of fibers, binders, and filler materials, varying in their combinations with the specifications required of the finished product. Generally I prefer to use the conventional paper making stocks, such as 55 kraft, sulphite, soda, rag or ground wood pulps, deriving these, if desired, from waste materials, such as old news, mixed papers, sulphite clippings, and old rags. With vegetable fibers may be combined various percentages of animal fibers, such as wool, or of 60 mineral fibers, such as asbestos.

Likewise, my process is not restricted to the use of any one type of organic binder. Asphalts, bitumens, pitches, natural resins, 65 such as rosin and shellac, and many kinds of synthetic resins can be employed. The one essential is that they be thermo-plastic and/or reducible under heat or conditions obtained in a suitable mixing device, to an 70 adhesive and viscous state. In using the so-called synthetic resins, certain precautions need to be exercised, as will be more fully developed hereinafter.

The selection of fillers is dictated by the 75 characteristics desired in the finished product, as is also the amount used. Color may, of course, be imparted by the use of pigments; increased dielectric strength may be obtained with particular fillers; special 80 molding properties with others, and the like.

The object of my invention is the production of a pulp of feltable fibers in suspension in a circulating medium with which a binder substance is associated, together with 85 a filler substance. Another object of my invention is the production of a novel type of association between the several substances which go to make up my pulp. Still another object of my invention is the 90 provision of a new and useful process for the employment of fillers in pulps which contain binder substances. Still another object of my invention is the production in felted articles of enhanced qualities derived 95 in part from the physical association of the ingredients which go to make up the pulp.

These and other objects of my invention which will be set forth hereinafter, or will be apparent to one skilled in the art upon 100

reading these specifications, I accomplish by that certain process and series of manipulations, and in that product of which I shall now describe an exemplary embodiment.

- 5 The particular objectives and advantages of my process may be illustrated with reference to the manufacture of sheets, boards or formed pulp products containing as the binder a synthetic resin such, for example, 10 as a one-stage creosol-formaldehyde resin. Within the classification of synthetic resins I would broadly include the condensation product of an aldehyde, the polymer of a hydrocarbon derivative, or the product of 15 the reaction between a polyhydroxy alcohol and an organic acid. This group comprises individual resinous substances of widely differing properties, and the adaptation of any one in particular must take into account 20 its properties with reference to the conditions of use in the present process and the proportion desired in the finished product. For example, the synthetic resins differ in point of time and temperature for conversion 25 under heat into their infusible and/or insoluble form. Generally those having a relatively long curing time are required when elevated temperatures are employed in the process of drying the resinous pulp 30 product, as, for example, in passing sheets over the heated drying drums of a paper machine. Combinations of these various synthetic resins in a felted fibrous structure can be converted under heat and pressure 35 into dense, so-called "laminated" phenolic products possessing great tensile strength, desirable electrical properties, resistance to moisture, and to the action of organic solvents and dilute acids.
- 40 Heretofore the base stock for laminated phenolic products has been made by saturating special papers, generally kraft or an absorbent cotton or purified wood cellulose paper, by passing it through a resin solution. The solvent is then evaporated by 45 means of heat, leaving the resinous matter coated upon and partially incorporated in the paper. From the papers so treated the various laminated products of this industry 50 have been made by stacking together either sheets or shapes cut therefrom to make a product of the desired thickness and cured between steam-heated platens in a hydraulic press at temperatures ranging from 140° to 55 200° centigrade, and under pressures of 1000 to 3000 pounds per square inch.

The present invention is concerned with a new method for securing a felted fibrous structure containing resin. The product 60 can be cured and pressed in equipment, and by the procedure now followed in the handling of paper sheets coated and partially saturated with resin. In other respects the product is quite novel, as will be understood 65 from what follows.

The method consists essentially in kneading together in a suitable mixer a mass of wetted cellulosic fibers and a liquid or semi-liquid resin, preferably reduced to this state by means of heat. When the cellulosic material, generally paper or a pulp, has been sufficiently broken, that is, defibrated, by the action taking place in the mixer, and the resin binder has been uniformly incorporated or distributed throughout the wet fibrous mass, more water is added. With continued mixing and heating, the fibers slowly absorb the water and the adhesive masses break down into a watery pulp which, with further refining as in a beater followed by Jordaning, can be reduced to the consistency required for forming on a cylinder screen, Fourdrinier wire, shape mold, or other pulp-forming device. In this manner sheets, boards or formed articles can be economically manufactured by conventional equipment. Essentially this is the process set forth in the co-pending application of Stevenson and Buron, Serial No. 468,454 referred to hereinabove.

Advantages inherent in this method, as compared with the processes of saturating paper and other webs with synthetic resins, which are at present in general use, comprise: (1) no solvents are required; (2) the resin is more uniformly distributed with respect to fiber surfaces; (3) sheets of any desired thickness can be made with resulting economies in pressing and molding; (4) cheaper fiber stock can be used, such, for example, as waste papers; (5) uncured scrap from trimming and the cutting out of irregular shapes can be completely salvaged; (6) less resin is required to secure the same degree of strength, density, and molding properties. All of these advantages are of practical importance.

In working with synthetic resins as well as other binders, I have carried this process one step further. It is now proposed to incorporate in compositions of this character, filler substances which are of non-fibrous or substantially non-fibrous character. A result of certain character may be obtained by mixing mineral fillers or the like with the pulp as it is being beaten or refined, as by adding such fillers to the paper mill beater. This has its disadvantages, however, residing primarily in that filler substance added to the beater is not homogeneously distributed throughout the body of the pulp, and insofar as it is brought into suspension therein, does not exhibit to any practical extent a stability of association therewith. It is therefore incompletely retained upon the screen when the fibers are felted together to form the finished product. As a consequence, much of it is lost, and the final product becomes nonuniform and may have a distinctly striated character.

By my present process I provide a practical means for incorporating mineral fillers with the synthetic resin in my exemplary embodiment, whereby the fillers become uniformly incorporated in the finished sheet, board or formed-up pulp, and are largely retained in the pulp as it is being de-watered and formed up. Broadly, in the practice of my invention, instead of adding the filler to the beater, I add the filler to the mixer wherein the binder is in an adhesive state, and wherein there is relatively so small a content of moisture, if any, as will not be effective in preventing the initial adhesion to, and incorporation of the filler in, the body of the binder. I prefer thoroughly to incorporate my filler with the binder in a liquid or semiliquid state before I incorporate the fibrous material therewith. By mixing my filler, usually substantially dry, with the binder substance, I can uniformly distribute the filler throughout the binder; and when I subsequently make my premix, i. e., when I add my wetted fibrous material to the mixer and incorporate it with the binder, and when I subsequently beat off the fibers and distribute them in a circulating medium, I find that the binder has the same relationship to the fibrous material in the finished pulp as hitherto, namely, it exists in minute, uncoated particles in stable relationship with the fibers; but it differs from binders hitherto employed by me in that it contains within its body and within the body of such particles as now constitute the binder, a substantial quantity of a mineral or other non-fibrous filler. In this way the filler is uniformly distributed, and is in a substantial degree adhesively associated with the binder, whereby, when the pulp is finally formed up, the filler material is very well retained therein.

With certain fillers and binders practically the same end result may be obtained by adding the filler to the mixer with, or immediately after, the wetted fibrous material, depending, I believe, in point of theory, upon the degree of relative ease with which a particular mineral filler is wetted by water or by the binder. If the filler, however, is one that is preferentially wetted by water it will not readily enter into an adhesive relationship to the binder and may appear in the final pulp in suspension quite independent of the binder. In such case the final result may be quite the equivalent of adding the filler to the beater at the pulping or refining stage. If there is a contact relationship between the filler and the binder in the finished pulp under these circumstances it appears to exist largely in a sporadic adhesion of particles of filler to the globules or fragments of binder which are, in considerable measure, in adhesive contact with the fibers in the final pulp.

With certain binders I have been able to incorporate by this procedure an amount of filler equal in weight to that of the binder, and substantially to retain both the binder and the filler in the stock when de-watered and formed upon a screen. This is indicated, however, by way of example, without implying an upper limit for filler incorporation. The filler need not be added dry to the binder material, but may be added wet, if desired, and the mixing continued to the point of driving out the greater part if not all of the water, prior to the addition of the fibrous material. The water should be driven out when following my preferred procedure, at least to the extent of bringing about an adhesive association between the filler and the binder. When mixing together filler and binder, it is not essential that any water be preserved in the mixer, as it is with the fibrous material in an advantageous procedure; since the combined binder and filler appears to act in the subsequent process steps for the formation of the pulp, substantially as a simple binder. Thus, while it is advisable not to carry on the mixing of the binder (with or without filler) and the fibrous material to the point of driving out all of the water in the mass, so as to preserve the avidity of the fibers for water, to preserve an incompletely coated condition of the fibers, and presumably to permit the formation of hydro-cellulose as the fibers are being beaten to form a pulp, the relationship of the filler to the binder is preferably that of a completely coated condition of the filler which is not thereafter alleviated.

In the instance of premixing a synthetic resin compounded with a mineral filler and cellulosic fibers, certain desirable properties are realized in the molding of pulp articles under heat and pressure. For example, a board so made, and prior to the curing of the synthetic resin, has the property of plastic flow even with relatively low percentages of binder. The lower limit can not be specified as it will vary with different resins; but properties of plastic flow have been noted in formed pulps made under my process, in which the resin constitutes less than 40% of the dry pulp by weight. Webs of fibrous material, such as paper or the like, which have been coated and/or saturated with a synthetic resin, may be pressed and cured, but they do not exhibit to any marked degree the properties of plastic flow under heat and pressure. If any substantial deformation is attempted, the web puckers or ruptures, and the desired result is not perfectly obtained. With premixed pulps, if the binder is in excess of the fibrous material, the quality of true plastic flow has been noted; but where the binder is relatively low in amounts, this property has not been per-

fefully developed. In a pulp made by my process, however, the filler serves to lubricate the mass, permitting a certain degree of flow in the fibers, and also facilitating the flow of the resin. Even with relatively low amounts of binder hereinabove referred to, I have found that my material is truly heat-plastic, and will flow and fill all of the interstices of a complicated mold. Thus, in 10 pressing under heat, the pressure is equalized, a much more homogeneous article results, and the final product is free of puckers, ruptures, knit lines, and the like.

Yet another advantage inherent in this 15 use of a mineral filler is increased mechanical strength in the pressed and cured articles made from this new resinous pulp.

The advantages, derived from the use of mineral fillers in resinous pulps, made in 20 accordance with my process, are not restricted to binders of the synthetic resin type, but are also to be noted in the use of other binders.

My process is, of course, of especial importance in the field of molded compositions containing synthetic resins, because here it is advantageous for a number of reasons, not the least of which is economic, to keep the amount of binder relatively low, 25 and to secure the mechanical reinforcement of a felted fiber structure. The range and utility of products which can be molded from sheeted fibrous stock containing synthetic resins has been greatly extended by 30 my invention.

As an example of a procedure in working with synthetic resins I may state the following: An exemplary resin suitable for my process may be prepared as follows:

40 Cresylic acid----- 39 pounds  
Phenol ----- 10 pounds  
Formaldehyde----- 47 pounds  
Ammonia----- 4 pounds

45 All of the ingredients are mixed together and heated in a steam-jacketed vacuum kettle equipped with a condenser, to a temperature of about 90° C., where the reaction starts and the temperature rises rapidly to 50 110° C. After about 20 minutes the reaction subsides whereupon heat is applied and the temperature maintained at 100° C. for about 40 minutes. Vacuum is then applied and heating continued. This removes the 55 water originally present in the formaldehyde and that formed by the condensation reaction. Heating is continued and the temperature slowly raised to 110° C. and held at this temperature until the resin has been 60 advanced to the proper stage, as shown by the hardness of the resin on cooling and by its rate of curing.

The rate of curing of the resin is determined by a hot plate test conducted as follows: A small amount of the resin is worked

with a spatula on a hot plate at 150° C. and its behavior noted and timed with a stopwatch. The resin first melts to a non-sticky liquid, then gradually becomes tacky and finally becomes rubbery and non-sticky.

By the described procedure a resin can be produced which becomes tacky in approximately 90 seconds, and becomes rubbery in approximately 250 seconds by the hot plate test.

The type of resin used is dependent upon the time and temperature used in drying the finished paper or board and the resin just described is an example of a resin suitable for use in heavy board which is to be dried in a Coe dryer or other apparatus which maintains a temperature between 100 and 125° C., under which condition the board becomes dry in approximately 2 hours.

For paper which is to be air-dried or dried at lower temperatures faster curing resins, such as those made with higher percentages of phenol, may be used. Care must be taken, however, to select a resin which will not become cured during the drying of the paper to the extent that it no longer has plastic flow under the heat and pressure condition used in molding.

This resinous material is placed in a suitable mixing or kneading machine, such as 95 the well-known Werner-Pfleiderer mixer, and under the influence of heat is brought to a semi-liquid or plastic condition. The desired quantity of mineral or other filler, say slate dust to the amount of 20% by 100 weight of the synthetic resin, is added thereto. As hereinabove explained, the nature and quantity of the mineral or other filler may be widely varied, and it is not necessary to describe a separate procedure with 105 varying fillers or varying amounts thereof. The filler may be added wet or dry. The rotation of the mixer blades is started, and in either instance mixing is carried preferably to the point of forming a homogeneous distribution of the filler material in the 110 binder. If the filler material has been added wet, it is advantageous to continue the mixing until the moisture has been driven out, and until the filler is not only completely incorporated in the body of the binder, but also in adhesive contact relationship therewith in all its parts. The filler will 115 preferably be in a completely coated condition.

After the incorporation of the filler into the binder material, the fibrous material which has been previously wetted with water, and which preferably contains approximately 50% by weight of water, is next 120 added. The fibrous material may substantially be in any amount desired.

For the production of a material which can be readily molded, as hereinabove described, a quantity of fiber can be used such 130

that the resulting pulp will have the following composition when computed upon the air-dry basis:

5 Resin..... 50 per cent  
Fiber..... 40 per cent  
Mineral filler..... 10 per cent

10 A suitable fiber furnish is one comprising equal weights (air-dry basis) of rag half stock and sulfite clippings. The use of some rag stock appears to be desirable in these compositions.

15 The binder containing the filler is kneaded together with the wet fibrous material in the presence of heat in a mixing machine, such as the familiar Werner-Pfleiderer mixer. After the binder and the fibrous material have been thoroughly mixed, but preferably before the water has been driven out 20 of the mass under the influence of heat, and while the fibers have substantially an incompletely coated condition and an avidity for water, the resultant mass in the mixer is broken down to a semi-pulp by the addition 25 of more water. This semi-pulp may then be transferred to a beater and beaten into a true pulp in which the fibers are fitted for felting, and are suspended in a quantity of water sufficient to act as a circulating medium. This pulp may be refined and/or 30 diluted as desired, and may be formed up upon the screen of a paper making machine or other pulp forming device. In it the binder exists in minute, uncoated particles 35 in stable and partial adhesive contact association with the fibers, with the binder particles themselves substantially containing the filler materials.

The formed and dried pulp will have the 40 characteristics, under heat, of plastic flow, and can be formed up under heat and pressure and cured to cause the resin to assume an infusible and/or insoluble condition. Prior to the treatment under heat and pressure, the resin should be largely in a secondary or incompletely cured condition, and any scrap which is the result of trimming or cutting the blanks for the pressing or molding operation, may be re-used in subsequent 45 batches of stock, preferably introduced at the premixing stage, or it can be shredded and used as a molding compound.

In working with other binder materials substantially the same procedure may be 50 followed. Thus, to an asphaltic substance such, by way of example, as those described in United States Patent No. 1,771,150, I may add in the mixer a desired quantity of a mineral filler, such as the slate dust or finely 55 ground silica, diatomaceous earth, or the like, and after thoroughly incorporating the two together, treat the combined mass as a binder, subsequently following through a procedure like that of the Stevenson and 60 Buron Patent No. 1,771,150. With other

binders than synthetic resins, and particularly with non-porous fillers, an equivalent increase in moldability results from the 70 filler incorporation, and, of course, with these other binders I achieve the other objects of my invention: substantially complete retention of the filler, and homogeneous distribution thereof.

Since the primary object in adding a mineral filler to a composition of synthetic resin 75 and a paper making fiber is to secure improved molding properties under heat and pressure for a minimum amount of resin contained therein, the proper selection of 80 filler and amount thereof is important. While for a given composition this factor can only be determined by experimentation, the use of absorbent materials, such as diatomaceous earths, is not recommended. Materials such as 200 mesh silica, finely ground 85 feldspar and paper makers' clay will generally be found satisfactory. When color is desired the filler may consist in part of pigments or lakes.

Having thus described my invention, what 90 I claim as new and desire to secure by Letters Patent, is:

1. A fibrous pulp in water suspension in association with a binder substance in particle form, the binder particles containing 95 filler materials in substantially homogeneous distribution therein.

2. A pulp of paper making fibers in suspension in a circulating medium, containing 100 binder particles in substantially homogeneous distribution, the said binder particles containing filler particles in substantially completely coated condition.

3. A pulp of feltable fibers in water suspension, and containing in stable association therewith a dispersed synthetic resin in combination with a pigmented mineral filler. 105

4. A pulp of feltable fibers in stable association with a dispersed synthetic resin containing a pulverulent mineral filler, and further characterized by freedom from uncombined mineral filler. 110

5. An uncoated composition of felted fibers containing in its interior and within the confines of its surface enough thermoplastic material to flow outwardly upon fusion under heat and pressure so as to form a continuous film wholly encasing the fibers and a mineral filler uniformly distributed 115 throughout said composition and dispersed 120 in said binder.

6. An uncoated composition of felted fibers containing in its interior and within the confines of its surface enough synthetic resin in an incompletely cured stage to flow 125 outwardly upon fusion under heat and pressure so as to form a continuous film wholly encasing the fibers and a mineral filler uniformly distributed throughout said composition and dispersed in said binder. 130

7. An uncoated composition of felted fibers containing in its interior and within the confines of its surface a synthetic resin in an incompletely cured state and a mineral 70  
5 filler, the particles of said filler being coated with and uniformly distributed in the resin material.
8. A molding composition comprising a structure of felted fibers and containing 75  
10 within its confines and in intrafiber distribution a mineral filler associated, as herein described, with a synthetic resin sufficient in quantity to flow outwardly upon fusion under heat and pressure to form a continuous 15 encasing film.
9. A molding composition comprising a structure of felted fibers and containing within its confines and in intrafiber distribution a mineral filler associated, as herein 20  
20 described, with a synthetic resin sufficient in quantity to flow outwardly upon fusion under heat and pressure to form a continuous 25 encasing film, and further characterized by the property of plastic flow under the conditions of molding.
10. A process of making a pulp which contains a binder and filler material, which comprises combining a filler material with the binder substance under conditions permitting 30  
30 an adhesive relationship between said substances, whereby the filler becomes completely coated with said binder, and associating the resulting binder with the fibrous material under conditions in which 35  
35 said fibrous material comes into adhesive contact with said binder material but is incompletely coated thereby, and subsequently dispersing the mass so formed in water to the extent of fitting the fibers therein for 40  
40 formation upon a paper machine screen.
11. A process of forming a pulp of fibrous material containing binder and filler substances, which comprises associating said binder and said filler substances under saturating 45  
45 conditions, and said binder and said fiber under non-saturating conditions, and subsequently dispersing the mass so formed in water sufficient to act as a circulating medium.
12. The process of making a pulp of fibrous material, binder and filler, which comprises associating said binder and said fiber under saturating conditions, and said binder and said fiber under non-saturating conditions but sufficient to bring about an adhesive 55  
55 relationship between the two, afterwards breaking down the said adhesive condition by the step of adding water as herein described and then dispersing the product so formed in water and beating the fibers to fit them for felting.
13. The process of preparing a fibrous pulp containing a filled plastic binder, comprising the steps of reducing said binder to a molten condition, incorporating therewith 60  
60 a pulverulent filler, and then adding thereto a quantity of wetted fibrous material, mixing under conditions to disperse the fibers, and thereafter adding to the mixer an additional amount of water sufficient to partially break up the adhesive masses of fiber and filled binder, and finally refining the resulting stock and diluting with water to a paper making consistency.
14. The process of preparing a fibrous pulp containing a filled synthetic resin, comprising the steps of reducing said resin to a molten condition, incorporating therewith a pulverulent filler, and then adding thereto a quantity of wetted fibrous material, mixing 65  
65 under conditions to disperse the fibers, and thereafter adding to the mixer an additional amount of water sufficient to partially break up the adhesive masses of fiber and filled binder, while maintaining temperature conditions throughout to preserve the resin in a substantially uncured state.
15. That process of forming a feltable pulp containing binder and filler substances, which comprises dispersing a filler in a binder and subsequently causing the said binder to adhere to fibrous materials in a pulp in water suspension, said binder existing in minute particles in said pulp and containing 70  
70 said filler material in dispersion.
16. A process of making fibrous pulps which comprises associating fibers, filler materials, and a binder under conditions insuring a complete coating of said filler material by said binder, but an incomplete coating of said fibrous material by said binder, and afterward dispersing the mass so formed in water, and beating the fibers to fit them for felting.
17. The process of making a pulp of fibrous material, polymerizable binder, and filler material, which comprises introducing a polymerizable binder in a secondary or incompletely polymerized stage into a mixing device and incorporating therewith a filler material to the extent of effecting a substantially homogeneous distribution of said filler in said binder, afterwards mixing with said mass wetted fibrous materials without completely coating the individual fibers thereof with said binder, adding water and mixing to form a semi-pulp, transferring said semi-pulp to a beater and beating the said semi-pulp to form a true pulp of feltable fibers with said binder and said filler in stable association therewith.
18. The process of making a pulp of fibrous material, synthetic resin and filler, which comprises mixing a filler material with said resin while in an incompletely polymerized stage to the extent of substantial homogeneous distribution, premixing the mass so formed with wetted fibrous material, and beating the resulting product to form a pulp.

19. The process of making a pulp of fibrous material, synthetic resin and filler, which comprises mixing a filler material with said resin in an incompletely polymerized stage to the extent of substantial homogeneous distribution, premixing the mass so formed with wetted fibrous material, and beating the resultant product to form a pulp, forming the said pulp upon a screen of a paper machine, drying the formed product, and polymerizing the resin therein under heat and pressure.

20. The process of making a pulp of fibrous material, synthetic resin and filler, which comprises mixing a filler material with said resin in an incompletely polymerized stage to the extent of substantial homogeneous distribution, premixing the mass so formed with wetted fibrous material, and beating the resultant product to form a pulp, forming the said pulp upon a screen of a paper machine, drying the formed product, and polymerizing the resin therein under heat and pressure in a closed mold, said polymerizing being accompanied by the plastic flow of said material to fill the interstices of said closed mold.

Signed at Cambridge, in the county of Middlesex, and State of Massachusetts, this 30 twenty-eighth day of February, 1931.

EARL P. STEVENSON.

35

40

45

50

55

60